

## UNITED STATES PATENT OFFICE

2,400,377

## COMPOSITION FOR TREATING KERATIN FIBERS

John Barber Speakman, Far Headingley, Leeds,  
England, assignor to Perm Ltd., Dover, Del.

No Drawing. Original application May 25, 1938,  
Serial No. 210,074. Divided and this applica-  
tion February 19, 1944, Serial No. 523,114. In  
Great Britain December 10, 1934

3 Claims. (Cl. 167—37.1)

This invention is concerned with compositions for use in the treatment of keratin containing fibers such as wool or hair.

The application is a divisional of my applica-  
tion Serial No. 210,074, filed May 25, 1938, (Pat-  
ent No. 2,351,718, issued 20th day of June, 1944),  
which is a continuation in part of Patent No.  
2,201,929, filed December 9, 1935.

Keratin containing fibers are customarily sub-  
jected to steaming or hot water treatment in the  
presence of compounds which may include re-  
ducing agents at or only slightly below the boil-  
ing point for the release of strain and the appli-  
cation of a permanent set.

It has been proposed to treat wool or hair with  
a boiling bisulphite solution while tensioning the  
wool or hair. Such treatment at the boiling  
point will result in disruption of the disulphide  
bonds of keratin and the immediate formation  
of S—NH bonds as indicated by the following  
equations:



where  $R—S—S—R$  and  $R'—NH_2$  represent the  
peptide and associated side chains of keratin.  
At or about the boiling point, the reactions take  
place with great readiness and a sufficient num-  
ber of linkages to impart a permanent set to the  
fibers is formed in so short a time that the proc-  
ess is commercially useful. At lower tempera-  
tures, however, the rate of formation of linkages  
as represented by Equation 2 above, is so small  
that a permanent set is not obtained in a rea-  
sonable time, and low-temperature setting is im-  
practicable.

The object of the invention is to provide a  
composition which will bring about release of  
strain in hair over a range of temperature, appre-  
ciably below the boiling point of water and es-  
pecially down through temperatures to as low as  
room temperature, where desired.

A further object of the invention is to provide  
a composition for treating keratin-containing  
fibers and causing disruption of the constituent  
disulphide bond of keratin, the composition com-  
prising a reducing agent of the group consist-  
ing of bisulphites and compounds capable of  
yielding bisulphites, together with a substantial  
quantity of a water soluble alcohol.

A further object of the invention is to provide  
a composition as set out in the preceding para-  
graph in which the water soluble alcohol is pres-

ent to the extent of 10 to 45 per cent. by weight.

The conditions for disruption of disulphide  
bonds of keratin are very favourable at about pH4,  
at which bisulphites and metabisulphites pro-  
duce pronounced fiber swelling, which favours  
relaxation and may be further developed by em-  
ploying a high content of an agent adapted to  
reduce ionisation of the salt and increase swell-  
ing, for example, a soluble alcohol, such as ethyl  
alcohol, glycerol, ethylene glycol or ethylene-  
glycolmonomethylether.

The composition of the invention brings about  
release of stress in hair by causing disruption of  
the disulphide bonds of keratin, the mechanism  
of the reactions being represented as follows, the  
symbols  $R—S—S—R$  and  $R'NH_2$  representing the  
peptide and associated side chains of keratin  
and  $NaHSO_3$  being employed as representative  
of alkali metal and ammonium bisulphites.



## Example

As indicated above bisulphites and metabisul-  
phites at pH4 are efficient in bringing about dis-  
ruption of the disulphide bond of keratin. In  
25 employing such reagents according to an ex-  
ample, the hair is treated with a 5 to 20 per cent.  
bisulphite or metabisulphite solution containing  
45 per cent. ethyl alcohol for about 15 minutes  
30 at room temperature or above. The solution may  
be removed by rinsing in plain warm water and  
the hair dried. If the composition is to be used  
in a preliminary step in the permanent waving  
35 of hair, the hair in the relaxed state and having  
many of the disulphide bonds broken is then  
wound on a curler or otherwise deformed, no sig-  
nificant internal stress developing. The config-  
uration given to the hair is then made permanent  
40 by treatment with a solution of an oxidizing agent  
such as a 10-volume hydrogen peroxide or a 10  
per cent. alkali metal persulphate solution, or  
the treatment with an oxidizing agent may follow  
treatment with the ketone or aldehyde solution  
for instance a 60% acetone solution.

45 Alternatively the configuration may be made  
permanent by treatment with an alkali which has  
not got pronounced reduced action such as so-  
dium carbonate solution, or ammonia in solu-  
tion or as a gas at room temperature or above, to-  
gether with or followed by oxidising agents. In  
50 this case, the alkali serves to depress swelling  
and promotes the action of the oxidising agent  
in forming disulphide bonds by oxidation of sul-  
phydryl groups.

55 The initial treatment of the hair with the bi-

sulphite or metabisulphite solution described above may also be given after the hair has been deformed, for example on a curler, and the same subsequent treatment given for making the set permanent.

The hair may then be given the usual after treatment of permanent waving operations.

Alternatively instead of winding the hair on curlers it is formed into waves or curls on the head after being moistened with the solution. To facilitate manipulation of the hair, a thickening agent may be added to the solution of reducing agent, for instance agar-agar or kieselguhr in sufficient amount to give the consistency of a paste. Suitable wetting agents may also be added.

The hair may then be given the usual finishing treatment of permanent waving operations.

In the application of the invention to fabrics made of keratins such as wool, the usual crumbing and blowing operations for the removal or equalising of stress in the fabrics may be replaced by a reduction treatment in cold or warm solutions of the composition. The fabrics may then be treated for the removal of the reducing agent, for example by washing, or, by means of an aqueous aldehyde or ketone solution and followed if desired by treatment with a solution of an oxidising agent such as a 10-volume hydrogen peroxide solution. Removal of the composition generally may be effected by treatment with an oxidising agent.

Stress may also be dissipated in the fibers by heating at as low a temperature as 37° C. with bisulphite solution containing, for example, 45 per cent. alcohol, and then if desired treating the

fibers with an oxidising agent with or without treatment with alkaline solution at a low temperature or exposure to an atmosphere containing volatile alkalies such as ammonia.

5 The invention may also be applied to the removal of distortion in knitted fabrics of wool, arising from uneven stress in the yarn, by treatment of the fabric with the composition at 37° C. followed by treatment with an oxidising agent, a treatment with an alkali being also possible where a bisulphite is used.

10 Yarns for the manufacture of curl fabrics or artificial astrakan and Persian lamb fabrics may have a permanent set given to them by treatment of the deformed yarn with the composition followed by treatment with an oxidising agent, a treatment with alkali in solution or as a gas being also possible where a bisulphite is used.

I claim:

20 1. A composition of matter for the treatment of keratin-containing fibers comprising a solution of an acid sulphite in water and an alcohol at about pH 4; the alcohol being present in quantities ranging from about 10 to 45% by weight of the solution.

25 2. A composition of matter as claimed in claim 1 and containing a thickening agent in amount sufficient to increase the viscosity of the solution.

30 3. A composition of matter for the treatment of keratin containing fibers comprising a solution of a reducing agent of the group consisting of bisulphites and compounds capable of yielding bisulphites in water and an alcohol at about pH 4, the alcohol being present in quantities ranging from 10 to 45% by weight of the solution.

JOHN BAMBER SPEAKMAN.